

## UNITED STATES PATENT OFFICE

1,938,646

PRODUCTION OF YARNS OR THE LIKE  
FROM ORGANIC DERIVATIVES OF CELLULOSE

William Ivan Taylor, Spondon, near Derby, England, assignor to Celanese Corporation of America, a corporation of Delaware

No Drawing. Application January 25, 1930, Serial No. 423,561, and in Great Britain February 5, 1929

25 Claims. (Cl. 18—54)

This invention relates to the production of filaments, threads, yarns, or other materials, such as ribbons, tapes, or straw capable of being produced by the extrusion of solutions of cellulose acetate or other organic derivatives of cellulose, the object of the invention being to produce such filaments, yarns, threads, ribbons, tapes, straw or the like, and likewise fabrics or articles containing them) of which the lustre is reduced or even 10 completely removed or which can readily be delustered.

The invention is characterized by the employment in the production of such materials (hereinafter referred to as "filaments") of Turkey red oil or other wetting agents whether comprising organic sulphonated acids or sulphuric esters or salts thereof, or otherwise, such wetting agents being employed in such a manner that the filaments produced are capable of having their lustre completely or partially removed by a treatment with moist steam or with aqueous, alcoholic, or other suitable liquids.

The invention is applicable to the production of filaments, by the dry or evaporative method or 25 by the wet or coagulation method. For example, in one method of carrying out the invention spinning solutions containing organic cellulose derivatives for use according to either of these methods may contain proportions of wetting agents such as, for example, soaps, sulphonated soaps, or sulphonated oils, it being understood, of course, that only such wetting agents are employed as are soluble in the solvent used in the spinning solution.

30 In the case of dry spinning a solution containing a wetting agent, the evaporation of the volatile solvent for the cellulose derivative from the extruded solution produces delustrable filaments having a content of the wetting agent. By treatment of the filaments with, for example, aqueous liquids, (preferably warm or hot) the filaments are delustered. The extent of the delustering can be determined by varying the amount of wetting agent added to the spinning solution, greater delustering requiring the use of larger proportions of the wetting agent. The steaming, or the aqueous or other treatment for the delustering of the filaments may be performed continuously with the dry-spinning of the filaments as by passing the 45 filaments through an aqueous or other suitable bath, or may be applied subsequently thereto. When forming a continuous operation with the dry-spinning process, the said treatment may be followed by a drying of the delustered filaments 50 and the dried filaments may be collected in any

convenient manner, such as by winding or twisting and winding.

In the spinning of solutions containing wetting agents as above described by the wet or coagulation method, the spinning bath is so chosen that 60 the filaments emerging from the bath contain a proportion of the wetting agent or agents and upon subsequent aqueous or other treatment become declustered.

Examples of wetting agents which may be employed in the production of delustered filaments according to the invention are salts of higher fatty acids, sulphonated higher fatty acids and salts thereof, naphthenic acids, naphthene sulphonate acids or aromatic sulphonate acids and salts thereof, 65 sulpho-aromatic fatty acids and salts thereof, resin soaps, sulphonated naphthalene formaldehyde condensation products, alkylated aromatic sulphonate acids such as iso-propyl or butyl naphthalene sulphonate acid, and salts thereof.

In the employment of aqueous liquors to carry out the reduction in the lustre of filaments which have received a content of a wetting agent according to the invention, it is preferred to carry out the treatment with heated liquors, though the 70 reduction in lustre may be effected, though more slowly by the action on the filaments of cold aqueous liquors.

The invention includes within its scope filaments, yarns, or threads containing wetting 75 agents and capable of being delustered by a subsequent treatment as indicated above, and also fabrics or articles made from or containing such filaments, yarns, or threads. The invention likewise includes filaments, yarns or threads produced in 80 the manner above described, and delustered by subsequent treatment with aqueous fluids. This treatment however may conveniently be deferred until the filaments, threads, or yarns have been worked into fabrics or articles, and may take 85 their place simultaneously with washing, dyeing, or other operations performed on the fabrics or articles.

Various methods of carrying out the invention will now be described in greater detail, with reference to the spinning of filaments of cellulose acetate, but it is to be understood that the following description is by way of illustration only and in no way limitative.

90 A spinning solution of cellulose acetate in acetone is given an addition of Turkey red oil, either during the mixing of the solution or after the cellulose acetate has dissolved. The solution is then extruded into a current of air in a spinning chamber, and the filaments produced are led out 95 100 105 110

- of the chamber and collected in any suitable manner, for example, by means of a cap-spinning device. The filaments contain a proportion of Turkey red oil and are steamed, or immersed in 5 or otherwise treated with water, preferably warm or hot, or alcohol, for the purpose of reducing the lustre.
- Turkey red oil in amounts varying from 1 to about 10 or 12% calculated on the weight of the 10 cellulose acetate has been found suitable for producing filaments varying in appearance from a mere dullness to a complete absence of lustre according to the amount of Turkey red oil employed.
- 15 Similar proportions of Turkey red oil may be used in spinning solutions from which the filaments are formed by the wet spinning process, a wet spinning bath of such a nature that the filaments emerging from the bath containing a portion of the Turkey red oil being employed.
- The term "filaments" in the appended claims is to be understood to cover extruded artificial products generally, i. e. filaments, yarns, threads, tapes, ribbon, straw or like products.
- 25 What I claim and desire to secure by Letters Patent is—
1. Process for the manufacture of delustrable artificial filaments which comprises extruding an organic solution of an organic derivative of cellulose containing a wetting agent into a setting medium which does not remove the wetting agent from the filaments so extruded.
  2. Process for the manufacture of delustrable artificial filaments which comprises extruding an organic solution of an organic derivative of cellulose containing a wetting agent which is a water soluble organic compound containing acid groups into a non-aqueous setting medium which does not remove the wetting agent from the filaments so extruded.
  3. Process for the manufacture of delustrable artificial filaments which comprises extruding an organic solution of cellulose acetate containing a wetting agent into a setting medium which does not remove the wetting agent from the filaments so extruded.
  4. Process for the production of delustrable artificial filaments which comprises extruding an organic solution of cellulose acetate containing a wetting agent which is a sulphonated organic compound into a non-aqueous setting medium in which the wetting agent is substantially undispersable.
  5. Process for the production of delustrable artificial filaments which comprises extruding an organic solution of cellulose acetate containing a sulphonated higher fatty acid into a non-aqueous setting medium in which the wetting agent is substantially undispersable.
  6. Process for the production of delustrable artificial filaments which comprises extruding an organic solution of cellulose acetate containing Turkey red oil into a non-aqueous setting medium in which the wetting agent is substantially undispersable.
  7. Process for the manufacture of delustrable artificial filaments, said process comprising extruding into an evaporative atmosphere an organic solution of cellulose acetate containing a wetting agent which is a water soluble organic compound containing acid groups, and causing the filaments so extruded to set in said evaporative atmosphere.
  8. Process for the manufacture of delustrable artificial filaments, said process comprising extruding into an evaporative atmosphere an organic solution of cellulose acetate containing a wetting agent which is a water soluble organic compound containing acid groups, and causing the filaments so extruded to set in said evaporative atmosphere.
- truding into an evaporative atmosphere an organic solution of cellulose acetate containing Turkey red oil, and causing the filaments so extruded to set in said evaporative atmosphere.
9. Process for the manufacture of artificial filaments having a reduced lustre which comprises extruding an organic solution of an organic derivative of cellulose containing a wetting agent into a setting medium in which the wetting agent is substantially undispersable, and subjecting the said filaments so formed to a treatment with an aqueous fluid. 80
10. Process for the manufacture of artificial filaments having a reduced lustre which comprises extruding an organic solution of an organic derivative of cellulose containing a wetting agent which is a water soluble organic compound containing acid groups into a non-aqueous setting medium in which the wetting agent is substantially undispersable and subjecting the said filaments so formed to a treatment with an aqueous fluid. 85
11. Process for the manufacture of artificial filaments having a reduced lustre which comprises extruding an organic solution of cellulose acetate containing a wetting agent which is a water soluble organic compound containing acid groups into a non-aqueous setting medium in which the wetting agent is substantially undispersable and subjecting the said filaments so formed to a treatment with an aqueous fluid. 90
12. Process for the production of artificial filaments having a reduced lustre which comprises extruding an organic solution of cellulose acetate containing a wetting agent which is a sulphonated organic compound into a non-aqueous setting medium which does not remove the wetting agent from the filaments so extruded and subjecting said filaments to a treatment with an aqueous fluid. 100
13. Process for the production of artificial filaments having a reduced lustre which comprises extruding an organic solution of cellulose acetate containing a sulphonated higher fatty acid into a non-aqueous setting medium which does not remove the wetting agent from the filaments so extruded and subjecting said filaments to a treatment with an aqueous fluid. 110
14. Process for the manufacture of artificial filaments having a reduced lustre, said process comprising extruding into an evaporative atmosphere an organic solution of cellulose acetate containing Turkey red oil, causing the filaments so extruded to set in said evaporative atmosphere and subjecting the set filaments to a treatment with an aqueous fluid. 115
15. Process for the manufacture of artificial filaments having a reduced lustre, said process comprising extruding into an evaporative atmosphere an organic solution of cellulose acetate containing a wetting agent which is a water soluble organic compound containing acid groups, causing the filaments so extruded to set in said evaporative atmosphere, and subjecting the set filaments to a treatment with an aqueous fluid. 120
16. Process for the manufacture of artificial filaments having a reduced lustre, said process comprising extruding into an evaporative atmosphere an organic solution of cellulose acetate containing Turkey red oil, causing the filaments so extruded to set in said evaporative atmosphere, and subjecting the set filaments to a treatment with an aqueous fluid. 125
17. Process for the production of artificial filaments having a reduced lustre which comprises extruding into an evaporative atmosphere an organic solution of cellulose acetate containing Turkey red oil, causing the filaments so extruded to set in said evaporative atmosphere, and subjecting the set filaments to a treatment with an aqueous fluid. 130
18. Process for the manufacture of artificial filaments having a reduced lustre, said process comprising extruding into an evaporative atmosphere an organic solution of cellulose acetate containing a wetting agent which is a water soluble organic compound containing acid groups, causing the filaments so extruded to set in said evaporative atmosphere, and subjecting the set filaments to a treatment with an aqueous fluid. 135
19. Process for the manufacture of artificial filaments having a reduced lustre, said process comprising extruding into an evaporative atmosphere an organic solution of cellulose acetate containing Turkey red oil, causing the filaments so extruded to set in said evaporative atmosphere, and subjecting the set filaments to a treatment with an aqueous fluid. 140
20. Process for the manufacture of artificial filaments having a reduced lustre which comprises extruding into an evaporative atmosphere an organic solution of cellulose acetate containing Turkey red oil, causing the filaments so extruded to set in said evaporative atmosphere, and subjecting the set filaments to a treatment with an aqueous fluid. 145
21. Process for the production of artificial filaments having a reduced lustre which comprises extruding into an evaporative atmosphere an organic solution of cellulose acetate containing Turkey red oil, causing the filaments so extruded to set in said evaporative atmosphere, and subjecting the set filaments to a treatment with an aqueous fluid. 150

extruding an organic solution of cellulose acetate containing a wetting agent which is a water soluble organic compound containing acid groups into a non-aqueous setting medium which does not remove the wetting agent from the filaments so extruded and subjecting the filaments continuously with their setting to a treatment with an aqueous fluid.

18. Process for the manufacture of artificial filaments having a reduced lustre, said process comprising extruding into an evaporative atmosphere an organic solution of cellulose acetate containing a wetting agent which is a water soluble organic compound containing acid groups, causing the filaments so extruded to set in said evaporative atmosphere, and subjecting the filaments continuously with their setting to a treatment with an aqueous fluid.

19. Artificial filaments of an organic derivative of cellulose susceptible to delustering under treatment with aqueous fluids, said filaments containing a wetting agent.

20. Artificial filaments of an organic derivative of cellulose susceptible to delustering under treatment with aqueous fluids, said filaments contain-

ing a wetting agent which is water soluble organic compound containing acid groups.

21. Artificial filaments of cellulose acetate susceptible to delustering under treatment with aqueous fluids, said filaments containing a wetting agent. 80

22. Artificial filaments of cellulose acetate susceptible to delustering under treatment with aqueous fluids, said filaments containing a wetting agent which is water soluble organic compound containing acid groups. 85

23. Artificial filaments of cellulose acetate susceptible to delustering under treatment with aqueous fluids, said filaments containing a wetting agent which is a sulphonated organic compound. 90

24. Artificial filaments of cellulose acetate susceptible to delustering under treatment with aqueous fluids, said filaments containing a sulphonated higher fatty acid compound. 95

25. Artificial filaments of cellulose acetate susceptible to delustering under treatment with aqueous fluids, said filaments containing Turkey red oil.

WILLIAM IVAN TAYLOR. 100

30

105

35

110

40

115

45

120

50

125

55

130

60

135

65

140

70

145

75

150